

1

2,983,742

DECOLORIZING AND IMPROVING METAL SALTS  
OF PARTIAL ESTERS OF DITHIOPHOSPHORIC  
ACIDS

Joseph Boba, Fort Lee, and Charles H. Kolker, Maplewood, N.J., assignors to Gulf Oil Corporation, Pittsburgh, Pa., a corporation of Pennsylvania

No Drawing. Filed Mar. 11, 1959, Ser. No. 798,612

10 Claims. (Cl. 260—429.9)

This invention relates to decolorizing and improving metal salts of partial esters of dithiophosphoric acid. Oil-soluble salts, especially polyvalent metal salts of O,O'-diesters of dithiophosphoric acid, have found extensive use in hydrocarbon lubricating oils because of their detergent, antioxidant, anticorrosion and antiwear properties. As is well known, these oil-soluble metal salts are conventionally prepared by reacting monohydric alcohols or phenols with phosphorus pentasulfide, usually in the mol proportion of 4:1, at temperatures in the range of 130° to 350° F. to form partial esters of dithiophosphoric acid, and then by reacting the thus-obtained partial esters with a basic metal compound at temperatures in the range of 60° to 280° F., to form the corresponding metal salts of the partial esters of dithiophosphoric acid.

It has been found that very often the oil-soluble metal salts prepared as described above will be objectionably dark in color, usually greenish, even when the reaction conditions are controlled carefully. The dark color is objectionable as it affects the marketability of the salts. Also the oil-soluble metal salts referred to above frequently exhibit a rather low pH, often less than 5, despite the use of equivalent or greater proportions of basic metal compound during salt formation. A low pH is objectionable in metal salts of partial esters of dithiophosphoric acids, as it affects the compatibility of the salts in lubricants with other improvement agents that have an alkaline pH.

It has now been found that the metal salts of partial esters of dithiophosphoric acids can be substantially decolorized and made less acidic by incorporation therein of a small amount of a trialkylolamine whose alkylol groups contain 1 to 4 carbon atoms each, whereby such salts are rendered more suitable for use as improvement agents in hydrocarbon oil lubricants. Excellent results have been obtained with triethanolamine, but other trialkylolamines of the class disclosed can be used. Excellent results are obtained with 0.2 to 0.75 percent by weight of the trialkylolamine but larger or smaller amounts can be used. For example, there can be used 0.05 to 1.0 percent by weight. The invention has been found especially advantageous in connection with zinc and calcium salts of diesters of dithiophosphoric acid such as the O,O'-diethyl esters, but it can be used in connection with other metal salts of other partial diesters of dithiophosphoric acid. For example, the invention can be used with alkali metal salts such as sodium and potassium salts, alkaline earth metal salts such as barium and strontium salts, other Group II (Mendelyeev's Periodic Table) metal salts such as magnesium salts, of partial esters of dithiophosphoric acid, such as di(2-ethylhexyl) dithiophosphoric acid, O,O'-di(cyclohexyl) dithiophosphoric acid, O,O'-di(methylcyclohexyl) dithiophosphoric acid. Examples of other partial esters are the O,O'-di-alkyl dithiophosphate esters of primary monohydric alcohols containing 3 to 20 carbon atoms per molecule, and the corresponding esters of phenols such as phenol and alkylated phenols such as cresol, octylphenol, nonyl-

2

phenol and the like. The present invention includes the process described as well as the product thereof.

Although the cause of the dark color in metal salts of dithiophosphate esters has not been definitely established, it is believed that such color arises from the presence of traces of heavy metals, principally iron, in the phosphorus pentasulfides, commercial grades of which frequently contain about 15 to 60 parts per million heavy metals calculated as sulfides. Nor has the mechanism by which decolorization takes place been conclusively determined. It is considered that the trialkylolamine forms complexes with the traces of heavy metal compounds in the dithiophosphate ester salt that are more stable than the uncomplexed metal compounds. However, this is somewhat negated by the fact that other agents capable of forming complexes with heavy metal compounds do not produce equivalent results.

The trialkylolamine employed in this invention need not be pure. For example, commercial mixtures containing mono- and di-alkylolamines can be used. However, the trialkylolamine employed in the present invention should contain less than about 50 percent of mono- and di-alkylolamines, as these materials are appreciably less effective than trialkylolamines for the purposes of this invention, and therefore necessitate the use of relatively larger proportions of the decolorizing agent. The use of larger proportions of the decolorizing agent is undesirable as such use imparts an objectionably large nitrogen content to the dithiophosphate.

30 Any amount of trialkylolamines that will improve the color of the dithiophosphate salts without adversely affecting other properties of the salts can be used. Any amount of the trialkylolamines that will produce a suitable improvement in color will also produce a useful improvement in pH. An appreciable improvement in color can be obtained by the use of as little as 0.05 percent trialkylolamine by weight of the metal salt. A major improvement is normally obtained by the use of proportions in the range of about 0.2 to 0.75 percent. However, 40 larger proportions can be used. For example, good results can be obtained with up to about 1.0 percent trialkylolamine. Proportions substantially greater than 1.0 percent are undesirable as such proportions unduly increase the nitrogen content of the dithiophosphate salts. The trialkylolamine is added to the dithiophosphate salts after the salt-forming reaction between the metal-containing base and the dithiophosphoric acid ester is complete. This is done in order to avoid preferential reaction of the trialkylolamine with the dithiophosphoric acid ester rather than color-forming components, and 50 in order that the metal content (derived from said base) of the salt will not be diminished.

The decolorizing reaction takes place spontaneously at ambient atmospheric temperatures and no further treatment is necessary. The trialkylolamine can be added in any convenient manner. Some agitation is desirable to insure thorough admixture of the materials, but this is not essential.

The effectiveness of the present invention was demonstrated upon a sample of a green plant-scale batch of calcium-zinc O,O'-di(Oxo octyl) dithiophosphate having a color greater than 1.5 ASTM union scale. To the sample there was added 0.5 percent by weight triethanolamine. The green color disappeared, and the color was lightened to less than 1.0 ASTM union.

60 In a specific embodiment of the invention O,O'-diethyl dithiophosphoric acid is prepared by adding 222 pounds (1 pound mol) phosphorus pentasulfide, containing 15 to 60 p.p.m. heavy metals, over a period of about four hours to about 533 pounds (approximately 4 pounds mols) of Oxo-octyl alcohol (mixed branched-chain octanols, mostly dimethylhexanols prepared by the Oxo

synthesis process) over a temperature range of 50 to 95° C., the temperature at the end of the reaction being about 90° to 95° C. The mixture is agitated several hours after addition of the phosphorus pentasulfide to complete the reaction. The resulting O,O'-diocetylthiophosphoric acid is then converted to salt form. Salt formation is effected by adding 1425 pounds (17.5 pound mols) zinc oxide to 11,900 pounds (33.6 pound mols) of O,O'-diocetylthiophosphoric acid, prepared as described above, at a starting temperature of 55° C. while maintaining a vacuum equivalent to 125 to 150 mm. Hg absolute pressure. The addition of zinc oxide is completed in about one hour, the temperature being allowed to rise to 85° C. during the addition. After all the zinc oxide is added the temperature is held at 80° to 85° C. for one hour to complete the reaction. Throughout the addition of the zinc oxide and during the one-hour holding period thereafter, nitrogen is bled into the reaction mass at a rate of 1000 to 1100 cu. ft. per hour. The reaction mass is then treated with about 150 pounds of methanolic hydrated lime. The batch of calcium-zinc O,O'-diocetylthiophosphate is then filtered through a precoated filter press. To the greenish product there is then added about 50 pounds (approximately 0.5 percent by weight) of a commercially-obtained triethanolamine. The color of the resulting product is lighter than 1.0 ASTM union, and the pH is greater than 5.

It will be understood that the invention is not limited to the metal salts or decolorizing agents of the foregoing embodiment and that other salts and other decolorizing agents referred to herein can be substituted for those in the foregoing embodiment in equivalent proportions in an obvious manner. For example, there can be used triisopropanolamine, tripropanolamine, and tri(2-ethyl, 2-hydroxyethyl)amine. Trimethanolamine can also be used where the consequent reduction in flash point is not objectionable.

As has been mentioned, the use of trialkylamines in accordance with the present invention improves the color of the metal salts of thiophosphoric acid esters and improves their compatibility in hydrocarbon oils with other addition agents. In addition, available experimental evidence shows that lubricating oils containing thiophosphate salts prepared in accordance with this invention do not produce increased engine deposits during engine operation as compared with oils containing conventional thiophosphate salts, and in fact, the former can tend to reduce such deposits. In addition, the advantages named are obtained without formation of undesirable colors, haze or the like, and without increasing the foaming tendencies or water-sensitivity, and without unduly increasing the nitrogen content of the salts.

It will be understood that many variations and modifications of the invention as described herein will readily suggest themselves to those skilled in the art, and that such modifications and variations can be resorted to without departing from the spirit of the invention, and that

the invention is limited only by the scope of the claims appended hereto.

We claim:

- 5 1. A process comprising incorporating a small amount, sufficient to reduce the color of the product, of a trialkylolamine whose alkylol groups each contain 1 to 4 carbon atoms, in a metal salt of a partial ester of thiophosphoric acid that contains an objectionable amount of color-forming components, said small amount being not greater than about 1.0 percent by weight of said salt.
- 10 2. The process of claim 1 where the trialkylolamine is triethanolamine.
- 15 3. The process of claim 1 where said small amount is about 0.05 to 1.0 percent by weight of said salt.
- 20 4. The process of claim 1 where said small amount is about 0.2 to 0.75 percent by weight of said salt.
- 25 5. The process of claim 1 where said metal is at least one member selected from the group consisting of zinc and calcium, and said partial ester is O,O'-diocetylthiophosphoric acid.
- 30 6. A process comprising reacting a member selected from the group consisting of monohydric alcohols and monohydric phenols with phosphorus pentasulfide that has an objectionable heavy metals content in the mol proportion of about 4:1, at a temperature in the range of about 130° to 350° F., to form a partial ester of thiophosphoric acid, reacting said partial ester with a basic compound of a metal selected from the groups consisting of alkali metals, alkaline earth metals, zinc and magnesium, at a temperature in the range of about 60° to 280° F. to form the corresponding metal salt of said partial ester, and incorporating in said salt a small amount, sufficient to reduce the color of the product, of a trialkylolamine whose alkylol groups each contain 1 to 4 carbon atoms, said small amount being not greater than about 1.0 percent by weight of said salt.
- 35 7. A composition comprising a major proportion of a metal salt of a partial ester of thiophosphoric acid that contains an objectionable proportion of color-forming components, and having combined therewith a small amount, sufficient to reduce the color of the salt, of a trialkylolamine whose alkylol groups each contain 1 to 4 carbon atoms, said small amount being not greater than about 1.0 percent by weight of said salt.
- 40 8. The composition of claim 7 where said trialkylolamine is triethanolamine.
- 45 9. The composition of claim 7 where said small amount is about 0.2 to 0.75 percent by weight of the salt.
- 50 10. The composition of claim 7 where said metal is at least one member selected from the group consisting of zinc and calcium, and said partial ester is O,O'-diocetylthiophosphoric acid.

#### References Cited in the file of this patent

#### UNITED STATES PATENTS

- 2,737,492 Beegle et al. \_\_\_\_\_ Mar. 6, 1956  
2,837,549 Reeves et al. \_\_\_\_\_ June 3, 1958

UNITED STATES PATENT OFFICE  
CERTIFICATE OF CORRECTION

Patent No. 2,983,742

May 9, 1961

Joseph Boba et al.

It is hereby certified that error appears in the above numbered patent requiring correction and that the said Letters Patent should read as corrected below.

Column 3, line 7, for "17.5" read -- 17.6 --.

Signed and sealed this 26th day of September 1961.

(SEAL)

Attest:

ERNEST W. SWIDER

Attesting Officer

DAVID L. LADD

Commissioner of Patents

USCOMM-DC